

1

2,865,796

**METHOD OF INCREASING STRESS CORROSION RESISTANCE OF ALUMINUM ALLOYS**Wilhelm Rosenkranz, Meinerzhagen in Westphalia,  
Eichholz, GermanyNo Drawing. Application October 11, 1956  
Serial No. 615,223

Claims priority, application Germany October 12, 1955

13 Claims. (Cl. 148—12.7)

The present invention relates to a method of increasing the corrosion resistance of aluminum alloys, and more particularly, it relates to a method of producing shaped aluminum alloy bodies having high corrosion resistance under conditions of stress.

The self-hardening properties of aluminum alloys containing about 4% of copper and between 0.5 and 1% of magnesium are well known, and aluminum alloys of the above composition have for many years played an important part in the production of workpieces formed by non-cutting shaping, such as aluminum alloy sheets, extrusions, forgings and the like. However, it became soon apparent that the above mentioned alloys are, due to their high copper content, of less corrosion resistance than other aluminum alloys. Especially in the case of aluminum alloy sheets of the above composition it has been attempted to overcome the disadvantage of low corrosion resistance by plating the alloy sheet with a corrosion resistant, copper free aluminum alloy, or, preferably, with pure aluminum. Thereby it could not be avoided that the strength of the sheet or the like was reduced in proportion to the thickness of the plating layer.

It has then been tried to utilize copperfree aluminum alloys containing about between 4% and 12% zinc and about between 1% and 6% magnesium. Such aluminum alloys possess improved strength properties as compared with aluminum alloys of the aluminum-copper-magnesium type. However, it was soon found out that the aluminum-zinc-magnesium alloys were subject to crack formation when being exposed simultaneously to mechanical stress and corrosive conditions. In other words, aluminum alloys of the type aluminum-zinc-magnesium show low resistance against stress corrosion, and for this reason such alloys could not be used to the desired extent in light metal construction for purposes for which these alloys, due to their great strength properties, would otherwise have been highly suitable.

The resistance of aluminum-zinc-magnesium alloys against stress corrosion was then improved by including elements such as chromium, vanadium or manganese in the alloy, which elements were supposed to prevent or at least considerably reduce the susceptibility against stress corrosion of workpieces formed of the last mentioned alloys by non-cutting shaping.

As is described in greater detail in my copending application Serial Number 560,890, now Patent 2,823,994, issued February 18, 1958, entitled "Aluminum Alloy and Workpiece," the customary testing for susceptibility to stress corrosion by means of the so-called fork-test does not give results which correspond to the effects of stress under corrosive conditions in the actual use of structural elements and other bodies obtained from aluminum alloys by non-cutting shaping.

Discrepancies between test results and actual performance can be eliminated by a testing method combining bent tests with exposure to atmospheric conditions. In carrying out this improved test method, T-profiles of the various aluminum alloys which are produced with ex-

2

trusion presses, are bent in the plane of the T-flange about the stem and then exposed to real or simulated atmospheric conditions. After more or less prolonged testing periods, the workpiece is examined for the appearance of the typical stress corrosion cracks which usually are formed in the once upset areas of the T-profile stem.

The results obtained in accordance with this improved testing method clearly show that even aluminum-zinc-magnesium alloys which have been stabilized with chromium, vanadium or manganese are far inferior with respect to stress corrosion resistance, to aluminum alloys of the aluminum-copper-magnesium type.

As fully disclosed in my copending application Serial Number 560,890, now Patent 2,823,994, issued February 18, 1958, above referred to, it has been found that great resistance against stress corrosion can be achieved by including a small percentage of silver in the aluminum-zinc-magnesium type alloy which also contains a small quantity of chromium and/or manganese and/or vanadium. However, the addition of silver to the aluminum alloy is frequently undesirable, primarily because of the relatively high costs thereof. It must be noted however, that excellent results have been obtained by subjecting a silver-containing aluminum alloy of the type described above to the method of the present invention as described further below.

It is an object of the present invention to overcome the above described difficulties in the production of high strength, stress-corrosion resistant aluminum alloy workpieces.

It is another object of the present invention to provide a method of producing shaped aluminum alloy bodies of high stress corrosion resistance consisting of an aluminum alloy of the aluminum-zinc-magnesium type.

It is yet another object of the present invention to increase the corrosion resistance under stress of shaped aluminum alloy bodies in an economical and easily controllable manner by suitably adjusting the temperature of the aluminum alloy body during the various heat treatments thereof.

With the above and other objects in view, the present invention mainly comprises in a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of the magnesium and of the zinc within the crystallites of the aluminum alloy body, the first temperature being so chosen as to maintain substantially the one metal in solution within the alloy thereby preventing precipitation thereof in the form of an intermetallic compound, and maintaining the aluminum alloy body during subsequent non-cutting shaping thereof at a temperature adapted to retain substantially the one metal in solution in the alloy, whereby a shaped aluminum alloy body of great stress corrosion resistance is formed.

In a preferred manner of carrying out the method of the present invention, the same comprises the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a pe-

riod of time sufficient to cause substantially equalization of concentration of the magnesium and of the zinc within the crystallites of the aluminum alloy body, the first temperature being so chosen as to maintain substantially the one metal in solution within the alloy thereby preventing precipitation thereof in the form of an intermetallic compound, adjusting the temperature of the aluminum alloy body to a second temperature sufficiently high to allow non-cutting shaping of the alloy body and not more than 20° C., higher than the first temperature, subjecting the aluminum alloy body to non-cutting shaping while the same is substantially at the second temperature, subjecting the thus shaped aluminum alloy body to solution heat treatment at a temperature not exceeding the first temperature by more than 50° C., quenching the heat treated shaped aluminum alloy body at room temperature, and subsequently hardening the same in boiling water, whereby a shaped aluminum alloy body of great stress corrosion resistance is formed.

It has been found that the method of the present invention will greatly increase the stress corrosion resistance of aluminum alloys which contain between 4% and 12% zinc, between 1% and 6% magnesium, at least one of the stabilizing elements chromium, vanadium and manganese in an amount of between 0.05% and 0.6%, preferably in an amount of between 0.15% and 0.25% chromium, 0.05% and 0.15% vanadium and 0.1% to 1.5% manganese. Most preferably the amount of manganese in the alloy is kept at about 0.8%, and the alloy may also contain in addition to the aforementioned essential constituents thereof, up to 2% copper and/or up to 1% silver plus the amounts of iron and silicon which are usually present as impurities in commercial aluminum.

When the resistance against stress corrosion of the above described alloys of the aluminum-zinc-magnesium type is tested by extruding the same in the shape of T-profiles, then bending in the plane of the T-flange about the stem and exposing to atmospheric conditions, it is found that typical stress corrosion cracks usually occur, while such stress corrosion cracks do not occur upon similar treatment of the lower strength alloys of the aluminum-copper-magnesium type.

It is well known that aluminum alloys are susceptible to stress corrosion only along the grain-boundaries which, in the case of aluminum-zinc-magnesium alloys in contrast to aluminum-copper-magnesium alloys, are electrochemically less noble than the mixed crystal. In view thereof it has now been attempted to produce workpieces of aluminum-zinc-magnesium alloys by non-cutting shaping in such a manner, i. e. with such a structure, that the corrosive attack is diverted from the grain boundaries. This can be achieved by forming in the crystallites structural constituents which are less noble than the grain boundaries.

Surprisingly it has been found that this can be achieved, according to the present invention by maintaining during heat treatment and non-cutting shaping of the aluminum alloy of the aluminum-zinc-magnesium type, which alloy also contains a small quantity of a stabilizer such as chromium, vanadium, manganese or another metal performing a similar function, definite temperature ranges as described further below.

The term "stabilizer" as used in the present application is meant to denote any one of the metals chromium, vanadium, manganese or of other metals performing the same function as the aforementioned metals within the alloy, or any combination of several of these metals.

It is essential in accordance with the present invention that the annealing or heat treatment of the aluminum alloy body prior to non-cutting shaping thereof is carried out at a temperature above the solubility temperature of the respective alloy, which temperature depends upon the contents of magnesium and zinc, as is

well known with the skill of the art, which temperature must also be such that substantially equalization of the concentration of the hardening alloy components zinc and magnesium takes place within the crystallites of the aluminum alloy body, while precipitation of the stabilizer metal which is present in a meta-stable solution, in the form of an intermetallic compound is prevented as far as possible. The thus achieved structural condition with respect to the stabilizer metal must then be maintained during transformation of the original aluminum alloy body or ingot into a shaped aluminum alloy body and also during heat hardening of the shaped body. Consequently, according to the present invention, the heating of the ingot which has previously been heat treated as described above, prior to deformation thereof, for instance by means of an extrusion press, must be carried out at a temperature which does not exceed the temperature of the previous heat treatment by more than 20° C. In order to prevent the precipitation of stabilizer metal-containing, for instance chromium-containing, compounds it has been found advantageous according to the present invention to carry out the second or predeformation heating of the aluminum alloy body by induction heating for a short period of time. The solution heat treatment of the shaped aluminum alloy body in a salt bath or the like must also be carried out at a temperature and for a period of time which will not cause precipitation of stabilizer metal-containing compounds. Consequently, according to the present invention, solution heat treatment is to be carried out at a temperature which at most exceeds the temperature of the pre-shaping first heat treatment by 50° C. The solution heat treatment too is preferably carried out for a relatively short period of time only. Solution heat treatment of the shaped aluminum alloy body is then followed in customary manner by quenching of the same at room temperature, preferably at about 15° C., and, finally, by hardening, preferably in boiling water, i. e. at a temperature of about 100° C.

By following the above described method of the present invention, a previously unattainable degree of stress corrosion resistance, as measured by the improved testing method described herein, is achieved. Optimum results are obtained when precipitation of stabilizer metal-containing compounds is not at all or only to a slight degree apparent in the finished shaped workpiece. However, even when the temperatures during the process of the present invention have not been controlled with sufficient accuracy so as to prevent precipitation of chromium or other stabilizer metal-containing compounds to a marked degree, the equalization of concentration of magnesium and zinc within the crystallites, and the reduction in the relative amount of the stabilizer metal which will precipitate, causes an improvement in the stress corrosion resistance of the workpiece, which, as stated above was so far not attainable with alloys of similar composition.

The specific narrow temperature ranges which are to be maintained according to the present invention in order to achieve highest stress corrosion resistance of the finished shaped workpiece, i. e., the temperature range for the heat treatment of annealing of the aluminum alloy ingots as well as the temperature range for the non-cutting shaping thereof depend to a considerable degree on the specific composition of the aluminum alloy and can easily be ascertained by simple tests which are well within the skill of the art.

The following examples are given as illustrative only of the method of the present invention, the present invention, however, not being limited to the specific details of the examples.

#### Example 1

Aluminum alloy ingots of the composition 4.53% zinc, 3.54% magnesium, 0.18% copper, 0.41% chro-

mium, 0.23% iron, 0.19% silicon and the balance aluminum, were annealed for six days at 460° C. and thereafter pressed into the shape of T-profiles. The temperature during the non-cutting shaping of the ingots was kept at about 420° C. The thus obtained T-profiles were subjected to solution heat treatment in a salt bath at 450° C. for 15 minutes and were subsequently hardened for 100 hours in boiling water.

Aluminum alloy ingots of the same composition were similarly treated, with the exception that the 6 days pre-shaping annealing treatment was omitted.

The T-profiles obtained with and without the pre-shaping annealing treatment were then tested for stress corrosion resistance according to the above described improved method.

Thereby it was found that the life span of the T-profiles formed from aluminum alloy ingots which had not been preheated varied in five tests between 4 and 53 days, while the T-profiles formed from aluminum alloy ingots which were preheated to 460° C. as described above withstood tests continuing for over 90 days.

#### Example 2

Comparison tests were carried out with an aluminum alloy having the following composition: 4.20% zinc, 3.60% magnesium, 0.97% copper, 0.20% chromium, 0.28% iron, 0.14% silicon and the balance aluminum. In test (a) T-profiles were formed without preceding heat treatment. In test (b) the aluminum alloy ingots were first heated for a period of 3 days to 450° C., and in test (c) the aluminum alloy ingots were first heated for a period of 3 days to 510° C.

The ingot temperature during extrusion of the T-profiles was kept in all experiments at 420° C., solution heating was carried out in all tests for 15 minutes in a salt bath of 450° C., and, also in all tests, the profiles were hardened for 100 hours in boiling water.

Thereafter, the T-profiles obtained in tests (a), (b) and (c) were examined by etching surface portions thereof, using for the etching of the surface portions nitric acid plus mixed solution according to Dix and Keller, and by being subjected to the improved method of testing for stress corrosion by bending under atmospheric conditions. The following results were obtained:

| Test     | Surface Etching                  | Life Span in Stress Corrosion Test |
|----------|----------------------------------|------------------------------------|
| (a)..... | Sharp Distinct grain boundaries. | between 4 and 43 days.             |
| (b)..... | grain boundaries not apparent.   | unbroken after more than 100 days. |
| (c)..... | sharp distinct grain boundaries. | between 57 and 82 days.            |

In the case of test (a) a primarily local recrystallization took place in that area of the crystallite of the original cast structure which due to crystal liquation had been impoverished with respect to alloy constituents. Since recrystallization in enriched areas under equal conditions proceeds more slowly, localized recrystallized areas are formed which are susceptible to stress corrosion. When, as in test (c), the cast structure is subjected to homogenizing heat treatment so as to equalize concentrations, whereby all or part of the chromium is precipitated in the form of an intermetallic compound, the tendency towards recrystallization is also greatly increased, so that in similar manner stress corrosion effects become apparent.

#### Example 3

Tests were carried out as more fully described in Example 2, however, with an aluminum alloy of the following, different composition: 4.09% zinc, 3.61% magnesium, 0.10% copper, 1.12% manganese, 0.28% iron, 0.07% silicon and the balance aluminum.

The life span of the T-profiles produced from the

above-described alloy under the conditions described in Example 2 was as follows:

| Test     | Life Span in Stress Corrosion Test |
|----------|------------------------------------|
| (a)..... | 5, 3, 5, 5 days.                   |
| (b)..... | unbroken after more than 100 days. |
| (c)..... | 5, 6, 4, 5 days.                   |

#### Example 4

Tests carried out according to Example 2 with an aluminum alloy of the composition: 4.19% zinc, 3.78% magnesium, 1.49% copper, 0.52% manganese, 0.24% iron, 0.12% silicon and the balance aluminum, gave results similar to those described in Example 3.

#### Example 5

An aluminum alloy containing large percentage amounts of alloying materials such as: 9.38% zinc, 2.07% magnesium, 0.16% copper, 0.32% chromium, 0.24% iron, 0.10% silicon and the balance aluminum, has high strength characteristics ( $\sigma_B=65-66 \text{ kg./mm.}^2$ ,  $\sigma_{0.2}=60-62 \text{ kg./mm.}^2$ ,  $\sigma_5=5\%$ ,  $H_B=185 \text{ kg./mm.}^2$ ).

T-profiles were produced from the above alloy according to the method of the present invention by first heating the ingots for a period of three days to a temperature of 430° C., extruding the profiles at an alloy temperature of 440° C., subjecting the extruded T-profiles to solution heat treatment for a period of 15 minutes in a salt bath having a temperature of 450° C., quenching at about 15° C., and subsequently hardening for 100 hours in boiling water.

The thus produced T-profiles were still unbroken after being tested for more than 100 days according to the improved method of testing stress corrosion resistance, while the life span of T-profiles produced from the same alloy and tested under the same conditions, but without the pre-shaping annealing treatment, or with pre-shaping homogenizing heat treatment at temperatures exceeding the permissible temperatures according to the present invention, showed varying shorter life spans, some as short as 6 days.

#### Example 6

Aluminum alloy ingots of the composition: 4.59% zinc, 2.95% magnesium, 0.09% copper, 0.22% chromium, 0.45% silver, 0.21% iron, 0.18% silicon and the balance aluminum were annealed for 72 hours at 420° C. Immediately prior to non-cutting deformation, the ingots were heated inductively for a short period of time to 430° C. Thereafter T-profiles were formed on an extrusion press of the heated ingots. The T-profiles were then solution heated at 450° C. in a salt bath for 15 minutes, quenched in water of room temperature, and subsequently hardened for 100 hours in boiling water.

Bend testing under atmospheric conditions according to the improved method for determining stress corrosion resistance, showed that the life span of the bent portions of the T-profiles exceeded 100 days.

The structure of shaped aluminum bodies produced according to the present invention shows after solution heating and subsequent quenching a typical reticulated and line forming pattern. This reticular structure is characteristic for the deformed, but not recrystallized supersaturated structural condition. It is probable that the boundaries within this reticular structure represent lattice-planes which were disturbed due to deformation of the alloy body and in which upon heating to suitable temperatures the elements magnesium, zinc and chromium collect which are present in oversaturating concentrations, while at higher temperatures precipitation of the chromium-containing phase takes place. The boundary planes of this reticular structure are electrochemically of very base quality, since they are dissolved under the influence of an acidic attacking medium, and thus exert a protective effect for the stress corrosion endangered.

grain boundaries. In case of recrystallization, however, this reticular structure disappears and consequently also its protective effect with respect to the grain boundaries.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of the invention and, therefore, such adaptations should and are intended to be comprehended within the meaning and range of equivalence of the following claims.

What is claimed as new and desired to be secured by Letters Patent is:

1. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic compound; and maintaining said aluminum alloy body during subsequent non-cutting shaping thereof at a temperature adapted to retain substantially said one metal in solution in said alloy, whereby a shaped aluminum alloy body of great stress corrosion resistance is formed.

2. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% and 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic compound; and maintaining said aluminum alloy body during subsequent non-cutting shaping and heat treatment thereof at a temperature adapted to retain substantially said one metal in solution in said alloy, whereby a shaped aluminum alloy body of great stress corrosion resistance is formed.

3. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic compound; adjusting the temperature of said aluminum alloy body to a second temperature sufficiently high to allow non-cutting shaping of said aluminum alloy body, to retain substantially said one metal in solution in said alloy and in

solution in said alloy and not more than 20° C. higher than said first temperature; subjecting said aluminum alloy body to non-cutting shaping while the same is substantially at said second temperature; and subjecting the thus-shaped aluminum alloy body to solution heat treatment at a temperature not exceeding said first temperature by more than 50° C. and such as to prevent any substantial precipitation of said one metal, whereby a shaped aluminum alloy body of great stress corrosion resistance is formed.

4. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermediate compound; adjusting the temperature of said aluminum alloy body to a second temperature sufficiently high to allow non-cutting shaping of said aluminum alloy body, to retain substantially said one metal in solution in said alloy and not more than 20° C. higher than said first temperature; subjecting said aluminum alloy body to non-cutting shaping while the same is substantially at said second temperature; subjecting the thus-shaped aluminum alloy body to solution heat treatment at a temperature not exceeding said first temperature by more than 50° C. and such as to prevent any substantial precipitation of said one metal; quenching said heat treated shaped aluminum alloy body at room temperature; and subsequently hardening the same in a hardening bath at about 100° C., whereby a shaped aluminum alloy body of great stress corrosion resistance is formed.

5. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermediate compound; adjusting the temperature of said aluminum alloy body to a second temperature sufficiently high to allow non-cutting shaping of said aluminum alloy body, to retain substantially said one metal in solution in said alloy and not more than 20° C. higher than said first temperature; subjecting said aluminum alloy body to non-cutting shaping while the same is substantially at said second temperature; subjecting the thus-shaped aluminum alloy body to solution heat treatment at a temperature not exceeding said first temperature by more than 50° C. and such as to prevent any substantial precipitation of said one metal; quenching said heat treated shaped aluminum alloy body at room temperature; and subsequently hardening the same in boiling water, whereby a shaped aluminum alloy body of great stress corrosion resistance is formed.

6. In a method of producing shaped aluminum alloy bodies having high corrosion resistance under conditions

of stress, the steps of annealing an aluminum alloy body consisting essentially of aluminum and between 4% and 12% of zinc, between 1% and 6% of magnesium, up to 1% of silver, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic compound; and maintaining said aluminum alloy body during subsequent non-cutting shaping thereof at a temperature adapted to retain substantially said one metal in solution in said alloy, whereby a shaped aluminum alloy body of great stress corrosion resistance is formed.

7. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, up to 2% copper, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic compound; and maintaining said aluminum alloy body during subsequent non-cutting shaping thereof at a temperature adapted to retain substantially said one metal in solution in said alloy, whereby a shaped aluminum alloy body of great stress corrosion resistance is formed.

8. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, up to 1% of silver, up to 2% of copper, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic compound; and maintaining said aluminum alloy body during subsequent non-cutting shaping thereof at a temperature adapted to retain substantially said one metal in solution in said alloy, whereby a shaped aluminum alloy body of great stress corrosion resistance is formed.

9. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, and between 0.05% and 1.5% of at least one stabilizer metal, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic com-

5 pound; and maintaining said aluminum alloy body during subsequent non-cutting shaping thereof at a temperature adapted to retain substantially said one metal in solution in said alloy, whereby a shaped aluminum alloy body of great stress corrosion resistance is formed.

10. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic compound; and adjusting the temperature of said aluminum alloy body prior to non-cutting shaping thereof for a short period of time to a temperature adapted to retain substantially said one metal in solution in said alloy and not exceeding said first temperature by more than 20° C.

11. In a method of producing shaped aluminum alloy bodies having high corrosion resistance under conditions of stress, the steps of annealing an aluminum alloy body consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being so chosen as to maintain substantially said one metal in solution within said alloy and to prevent substantially precipitation thereof in the form of an intermetallic compound; and adjusting the temperature of said aluminum alloy body to a second temperature sufficiently high to allow non-cutting shaping of said aluminum alloy body, to retain substantially said one metal in solution in said alloy and not more than 20° C. higher than said first temperature; subjecting said aluminum alloy body to non-cutting shaping while the same is substantially at said second temperature; subjecting the thus-shaped aluminum alloy body to solution heat treatment at a temperature not exceeding said first temperature by more than 50° C. and such as to prevent any substantial precipitation of said one metal; quenching said heat treated shaped aluminum alloy body 55 at a temperature of about 15° C.; and subsequently hardening the same in boiling water.

12. In a method of producing shaped aluminum alloy bodies having high corrosion resistance under conditions of stress, the steps of annealing an aluminum alloy body 60 consisting essentially of aluminum and between 4% and 12% of zinc, between 1% and 6% of magnesium, at least one metal belonging to the group consisting of chromium, vanadium and manganese, in amounts of between 0.05% and 0.6% chromium, 0.05% and 0.15% vanadium and 0.1% to 1.5% manganese, the zinc content of said alloy being greater than the magnesium content thereof, at a first temperature and for a period of time sufficient to cause substantially equalization of concentration of said magnesium and of said zinc within 65 the crystallites of said aluminum alloy body, said first temperature being so chosen as to maintain substantially said one metal in solution within said alloy and to prevent substantially precipitation thereof in the form of an intermetallic compound; and maintaining said 70 aluminum alloy body during subsequent non-cutting shap-

11

ing thereof at a temperature adapted to retain substantially said one metal in solution in said alloy, whereby a shaped aluminum alloy body of great stress corrosion resistance is formed.

13. In a method of producing shaped aluminum alloy bodies having high corrosion resistance under conditions of stress, the steps of annealing an aluminum alloy body consisting essentially of aluminum and between about 4% and 10% of zinc, between about 2% and 4% of magnesium, and at least one metal belonging to the group consisting of chromium, vanadium and manganese, in amounts of between 0.05% and 0.6% chromium, 0.05% and 0.15% vanadium and 0.1% to 1.5% manganese, at a first temperature and for a period of time sufficient to cause substantially equalization of concentration of said magnesium and of said zinc within the crystallites of said aluminum alloy body, said first temperature being

10

15

12

so chosen as to maintain substantially said one metal in solution within said alloy and to prevent substantially precipitation thereof in the form of an intermetallic compound; and maintaining said aluminum alloy body during subsequent non-cutting shaping thereof at a temperature adapted to retain substantially said one metal in solution in said alloy, whereby a shaped aluminum alloy body of great stress corrosion resistance is formed.

## References Cited in the file of this patent

## UNITED STATES PATENTS

|           |                   |               |
|-----------|-------------------|---------------|
| 2,165,441 | Beck et al. ----- | July 11, 1939 |
| 2,736,674 | Harmon -----      | Feb. 28, 1956 |

## FOREIGN PATENTS

|         |                     |               |
|---------|---------------------|---------------|
| 438,512 | Great Britain ----- | Nov. 11, 1935 |
|---------|---------------------|---------------|